

## UNITED STATES PATENT OFFICE

JOSEPH KENT SMITH, OF DETROIT, MICHIGAN, ASSIGNOR TO BERYLLIUM DEVELOPMENT CORPORATION, OF NEW YORK, N. Y., A CORPORATION OF DELAWARE

## COPPER ALLOY

No Drawing. Application filed December 22, 1931. Serial No. 582,662.

This invention relates to alloys of great strength, extreme toughness, and resistance to corrosion, such alloys being particularly suitable for condenser tubes and similar uses where somewhat elevated temperatures are involved.

The alloys of my invention represent a copper base, copper comprising at least 70% and no more than 90% of the total. The other major element present is nickel, which comprises the greater portion of the remainder of the alloy. The alloys of the series differ from standard copper-nickel types in that they contain relatively small, but nevertheless very important, percentages of beryllium and manganese. The content of each of these last two metals should be at least 0.1% and no greater than 2% of the total weight of the alloy, preferably with more beryllium than manganese.

In addition to the four elements present as listed above, there will inevitably also be present impurities arising out of the constituent metals, such as iron, etc.; such impurities should, however, not exceed 0.5% in total.

As an example of my invention, I can cite an alloy comprised as follows:

|                        | Per cent |
|------------------------|----------|
| 30 Copper              | 79.5     |
| Nickel                 | 19.5     |
| Beryllium              | 0.5      |
| Manganese              | 0.25     |
| Constituent impurities | 0.25     |

35 This alloy is particularly well adapted for condenser tube use and for similar utilization where the above mentioned factors of strength and resistance to corrosion are vital.

40 The percentages are by weight.

I claim:

1. An alloy approximately consisting of copper 70 to 90%, nickel 10 to 30%, beryllium 0.1 to 2.0%, and manganese 0.1 to 2.0%.
- 45 2. An alloy approximating 79.5% of copper, 19.5% of nickel, and 0.5% of beryllium and 0.25% of manganese.

In testimony whereof I have hereunto signed my name.